

## UNITED STATES PATENT OFFICE

1,963,627

## EXPLOSIVE COMPOSITION

Harold A. Lewis, Woodbury, N. J., and Clifford A. Woodbury, Media, Pa., assignors to E. I. du Pont de Nemours & Company, Wilmington, Del., a corporation of Delaware

No Drawing. Application April 2, 1932,  
Serial No. 602,809

14 Claims. (Cl. 52—11)

This invention relates to an improvement in explosive compositions having a liquid explosive ingredient as a sensitizing agent, and in particular to a composition of the permissible type comprising as an ingredient a carbonaceous combustible material consisting of a treated cereal grain which has previously been expanded by subjection to high pressure and subsequent sudden release of said pressure.

10 The advantages of low density dynamites have become very great in recent years particularly for the blasting of materials having relatively low resistance. By means of these low density compositions the strength of the explosive is well distributed thus preventing unnecessary shattering of the material to be blasted. These and many other advantages of low density dynamites of various types are clearly described in the prior art. Heretofore the more desirable types of these 20 low density dynamites have been produced by means of various carbonaceous combustible ingredients principal among which have been balsam pith, balsa wood, ground cornstalks, etc.

An object of this invention is a low density 25 dynamite containing as an ingredient an improved combustible material. A further object is to provide a low density dynamite of improved sensitiveness properties over prior art compositions by means of a combustible ingredient having relatively low absorbent properties for liquid explosive materials. A still further object of our invention is an explosive composition containing as an ingredient a treated cereal grain which has been previously expanded by subjection to 35 high pressure and subsequent sudden release of said pressure. Other objects will appear as the description proceeds.

These objects have been accomplished by the following invention in which we have found that 40 a very desirable explosive may be made by means of certain treated cereal grains which have been artificially expanded or puffed, and particularly that form expanded by subjection to high external and internal pressure and subsequent sudden 45 release of said pressure.

We have found furthermore that various cereal grains which lend themselves readily to this treatment will accomplish our purpose such for example as wheat, rice, etc. Various methods 50 may be used to accomplish this treatment but in any case the cereal grain remains intact except that it is considerably enlarged and the material thereof has been changed greatly in density. In such treatment the pressure applied from without permeates the material of the grain and when

the external pressure is released the pressure within the grain walls causes the explosion or puffing of the grain kernel, thus resulting in a light, fluffy material. In order to convert this material into suitable form for our purpose the 60 expanded cereal grains are ground, crushed, or otherwise disintegrated so as to make the material readily combustible in explosive compositions. We prefer, however, to cut the material to obtain the proper form, in order not to destroy 65 the low density properties existing in the original puffed grain.

Material of a suitable size for our purpose may be obtained if care is taken that the grain particles are not too small in size. We have found that 70 a suitable material has preferably a size such that a major portion will pass a 6-mesh screen and at the same time be held on a 60-mesh screen.

U. S. Patent 1,687,023 to N. G. Johnson and 75 S. G. Baker covers an explosive composition containing as a combustible ingredient ground popped corn. The distinction between that patent and the present invention will at once be apparent, the present material comprising an expanded grain which derives its expanded condition by the application of high pressure of a vapor, such as steam, and the sudden release of this pressure.

This explosive ingredient according to our invention has a density varying between 0.09 and 0.15 85 depending on the method of treating the cereal grains. Dynamite compositions containing this ingredient have superior properties over compositions containing other ingredients of equally low density. The finished explosive compositions 90 containing this puffed cereal material are not only low in density but have excellent sensitiveness qualities by reason of the combustible material having low absorption properties for nitroglycerin or other liquid explosive ingredient or ingredients.

Our invention is applicable to all non-gelatinous types of dynamite compositions. The three main classes are commonly known as straight dynamites, ammonia or extra dynamites, and permissible dynamites. The straight dynamites are produced in strengths varying from about 20 to 75% and are used in blasting work where high velocity and sensitiveness to detonation are essential. They ordinarily comprise a liquid explosive ingredient equal in percentage to their grade strength, combustible absorbents and sodium nitrate. The ammonia dynamites are likewise made in several strengths and are used for general blasting. They comprise a lower per- 100 105 110

centage of liquid explosive than the straight dynamites of similar grade and contain also ammonium nitrate, sodium nitrate and combustible absorbents. The 20% ammonia dynamite, for example, may contain 10 to 15% of liquid explosive and 8 to 15% ammonium nitrate, while the 60% ammonia dynamite may have 15 to 30% of liquid explosive and 45 to 60% ammonium nitrate. The permissible dynamites are ordinarily 10 of high grade strength, from 40 to 70%, and are intended for use in coal mines where there is danger of explosion from mine gases and coal dust. These contain relatively low percentages of liquid explosives, ordinarily between 8 and 15%, and 15 relatively high percentages of ammonium nitrate, 60 to 80%, combustible absorbents, and in many cases inorganic salts for the purpose of reducing the flame temperature, sodium chloride or sodium nitrate for example.

20 The following examples are given to further illustrate the foregoing explosives but the invention is applicable equally well to many different types of explosives as will be apparent.

|                          | Percent | Percent | Percent |
|--------------------------|---------|---------|---------|
| Nitroglycerin.....       | 10      | 60      | 23      |
| Ammonium nitrate.....    | 75      | 52      |         |
| Sodium nitrate.....      | 5       | 20      | 14      |
| Puffed cereal grain..... | 8       | 5       |         |
| Other combustible.....   | 2       | 15      | 2       |
|                          |         |         | 9       |

In addition to the improvement in other properties, the low density effect of the use of our new combustible ingredient is shown by the fact that it makes possible the production of straight and ammonia dynamites on otherwise standard formulas, weighing less than 181 grams per  $1\frac{1}{4} \times 8''$  cartridge against a weight of 210 to 220 grams previously obtained. Similarly with dynamites of the permissible type, with the new ingredient, weights of  $1\frac{1}{4} \times 8''$  cartridges less than 146 grams may be obtained, much lower densities being possible with complete utilization of the treated expanded cereal grains.

It will be understood of course that we may vary widely the percentages of ingredients shown in the examples given and may introduce additional ingredients without departing from the spirit of the invention. We prefer, however, to use an amount of treated cereal grain varying between 1 and 20%, since less than 1% of this material will not have the desired effect on the density, while more than 20% will be undesirable because of the effect on the sensitiveness of the powder. The exact amount of our treated cereal product for use will depend on the proportions of the other ingredients present in the dynamite and on the density and other properties desired. Preferably, not less than 5% of nitroglycerin will be incorporated in my improved explosive composition, since a smaller amount than this will not have the desired sensitizing effect. We may use in place of nitroglycerin, for example, solutions in nitroglycerin of various materials commonly considered as freezing point depressants, nitroglycol, nitrated polymerized glycerin, nitrated sugars, nitrocompounds, etc. The amount of sodium nitrate may likewise be increased or decreased as desired, or omitted entirely, in which case sodium chloride or other flame suppressing material may be used. Similarly, we may use, together with the treated puffed cereal grain, high density combustible materials such as cornmeal, ivory nut meal, flour,

etc., or other low density carbonaceous materials, such as bagasse pith, ground cornstalks, etc.

It is therefore to be understood that we are to be limited in our invention only as indicated in the following patent claims.

We claim:

1. An explosive composition characterized by low density, which comprises a liquid explosive ingredient as sensitizing agent, and a low density, combustible ingredient comprising comminuted particles of puffed cereal grain, the structure of whose starch granules has been disrupted substantially throughout the mass of the same. 85

2. An explosive composition characterized by low density which comprises nitroglycerin as sensitizing agent, and a low density combustible ingredient comprising comminuted particles of puffed cereal grain, the structure of whose starch granules has been disrupted substantially throughout the mass of the same. 90

3. An explosive composition characterized by low density, which comprises more than 5% of a liquid explosive ingredient as sensitizing agent, and a low density, combustible ingredient comprising comminuted particles of puffed cereal grain, the structure of whose starch granules has been disrupted substantially throughout the mass of the same. 95

4. An explosive composition characterized by low density, which comprises a liquid explosive ingredient as sensitizing agent, and at least 1% of a low density, combustible ingredient comprising comminuted particles of puffed cereal grain, the structure of whose starch granules has been disrupted substantially throughout the mass of the same. 100

5. An explosive composition of the permissible

type characterized by low density which comprises a liquid explosive ingredient, ammonium nitrate, a non-explosive salt adapted to reduce flame temperature, and a low density combustible ingredient comprising comminuted particles of puffed cereal grain, the structure of whose starch granules has been disrupted substantially throughout the mass of the same. 115

6. An explosive composition of the permissible

type characterized by low density, which comprises a liquid explosive ingredient, ammonium nitrate, a non-explosive salt adapted to reduce flame temperature, and a low density, combustible ingredient comprising comminuted particles of puffed cereal grain, the structure of whose starch granules has been disrupted substantially throughout the mass of the same, said composition having a density such that a  $1\frac{1}{4} \times 8''$  cartridge weighs less than 146 grams. 120

7. An explosive composition of the straight dynamite type characterized by low density, which

comprises a liquid explosive ingredient, sodium nitrate, and a low density, combustible ingredient comprising comminuted particles of puffed cereal grain, the structure of whose starch granules has been disrupted substantially throughout the mass of the same. 135

8. An explosive composition of the straight dy-

namite type characterized by low density which comprises a liquid explosive ingredient, sodium nitrate, and a low density combustible ingredient comprising comminuted particles of puffed cereal grain, the structure of whose starch granules has been disrupted substantially throughout the mass of the same, said composition having a density such that a  $1\frac{1}{4}'' \times 8''$  cartridge weighs less than 181 grams. 145

9. An explosive composition of the ammonia 150

- dynamite type characterized by low density, which comprises a liquid explosive ingredient, ammonium nitrate, sodium nitrate, and a low density, combustible ingredient comprising comminuted particles of puffed cereal grain, the structure of whose starch granules has been disrupted substantially throughout the mass of the same. 80
10. An explosive composition of the ammonia dynamite type characterized by low density, which comprises a liquid explosive ingredient as sensitizing agent, ammonium nitrate, sodium nitrate, and a low density, combustible ingredient comprising comminuted particles of puffed cereal grain, the structure of whose starch granules has been disrupted substantially throughout the mass of the same, said composition having a density such that a  $1\frac{1}{4}'' \times 8''$  cartridge weighs less than 181 grams. 85
- 15 11. An explosive composition characterized by low density which comprises a liquid explosive ingredient as sensitizing agent, and 1 to 20% of a low density combustible ingredient comprising comminuted particles of puffed cereal grain, the structure of whose starch granules has been disrupted substantially throughout the mass of the same. 90
- 20 12. An explosive composition characterized by low density, which comprises more than 5% of a liquid explosive ingredient as sensitizing agent, 95
- 25
- 30
- and at least 1% of a low density, combustible ingredient comprising comminuted particles of puffed cereal grain, the structure of whose starch granules has been disrupted substantially throughout the mass of the same, said composition having a density such that a  $1\frac{1}{4}'' \times 8''$  cartridge weighs less than 181 grams. 100
13. An explosive composition characterized by low density, which comprises nitroglycerin as a sensitizing agent, and a low density, combustible ingredient comprising comminuted particles of puffed cereal grain, the structure of whose starch granules has been disrupted substantially throughout the mass of the same, said cereal grain being present in the explosive in such degree of fineness that more than 50% of the material will pass a 6-mesh and be retained on a 60-mesh screen. 105
14. An explosive composition characterized by its low density, which comprises a liquid explosive ingredient and 1 to 20% of a low density, combustible ingredient comprising comminuted particles of puffed cereal grain, the structure of whose starch granules has been disrupted substantially throughout the mass of the same, said cereal grain being present in the explosive in such degree of fineness that more than 50% of said grain will pass a 6-mesh screen and be retained on a 60-mesh screen. 110

HAROLD A. LEWIS.

CLIFFORD A. WOODBURY.

105

|    |     |
|----|-----|
| 35 | 110 |
| 40 | 115 |
| 45 | 120 |
| 50 | 125 |
| 55 | 130 |
| 60 | 135 |
| 65 | 140 |
| 70 | 145 |
| 75 | 150 |